

1

3,153,687

**PRODUCTION OF VISCOSE RAYON**  
Brewster Blanton Eskridge, Candler, N.C., assignor to  
American Enka Corporation, Enka, N.C., a corpora-  
tion of Delaware  
No Drawing. Filed Jan. 17, 1962, Ser. No. 166,908  
4 Claims. (Cl. 264—191)

This invention relates generally to the manufacture of rayon threads, fibers, yarn and the like products herein-after referred to collectively as yarn and more particularly to the production of high modulus viscose rayon yarn characterized by its high strength and low elongation values making it especially suitable for use in rug backing and in reinforcing rubber products such as belting and the like.

Yarn having high strength and low elongation values is commonly referred to as high modulus yarn. The modulus of yarn is determined by the following formula:

$$M = \frac{100S}{E}$$

wherein M is modulus, S is break strength in grams per denier, and E is percent of elongation. Accordingly, in order for yarn to have a high modulus, it must have a high breaking strength and an attendant low percentage of elongation.

In an effort to obtain high modulus rayon yarn, numerous modifications in rayon manufacturing processes have been proposed wherein various combinations of modifiers and other additives are employed at miscellaneous stages during the production of the yarn.

A process of particular significance is that disclosed in application Serial No. 740,189, having common ownership herewith, wherein a viscose containing an ethoxylated amine modifier is extruded into an acid spinning bath. The threads thus-produced are then aftertreated by passing them through a cold intermediate bath containing formaldehyde, and then through a hot stretch bath. In another process, disclosed in U.S. Patent No. 3,007,766, a viscose containing an alkali metal salt and modifiers, such as polyethylene glycol, ethoxylated amines and their quaternized derivatives is extruded into an acid spinning bath followed by passing the thus-produced threads through an intermediate bath containing formaldehyde and then through a hot acid stretch bath also containing formaldehyde.

While the use of formaldehyde in an intermediate and third bath imparts improved properties to the threads, in that they possess a higher moduli than that obtainable solely with the use of modifiers in combination with a cold intermediate bath, there are nevertheless certain disadvantages to its use in this manner. The cost of installing and maintaining an intermediate bath is a major factor in the expense of such a high modulus system. Furthermore, formaldehyde vapors escaping from the baths create extremely unsatisfactory operating conditions for workers employed in plants using this system due to objectional odors and disagreeable effects thereby produced. Moreover, consumption of formaldehyde is high, which increases the operating costs of this system.

Accordingly, it is an object of this invention to provide a process for manufacturing high modulus viscose rayon

2

yarn not having the disadvantages inherent in the known processes.

An additional object of this invention is to provide a simple and economical process for producing high modulus viscose rayon yarn.

Another object is to provide a process for producing high modulus viscose rayon yarn having high strength and low elongation values.

A still further object of this invention is to provide a process for producing viscose rayon yarn utilizing a novel combination of modifiers whereby a viscose rayon yarn with improved physical properties is produced.

These and other objects will become apparent from the following detailed description.

It has been discovered that the above objects may be accomplished by introducing small amounts of a lower aliphatic aldehyde into the viscose under certain critical conditions, thereby eliminating the aldehyde containing intermediate bath and the disadvantages and expense incidental thereto. In accordance with this invention, high modulus viscose rayon yarn having a high breaking strength and low elongation is obtained when a small amount of formaldehyde is introduced into the viscose in addition to other known modifiers. The addition of the

formaldehyde should be carried out in an indirect manner by adding it to the caustic soda solution (dissolving lye) for the cellulose xanthate crumbs. This should be done immediately prior to the addition of the crumbs to the solution, thereby assuring uniform dispersion throughout the resulting viscose solution. It is very critical that the formaldehyde be thoroughly mixed with viscose and that it be added to the viscose indirectly through the dissolving lye. Adding it to the viscose at any subsequent stage of processing prior to spinning will not produce as high a modulus yarn as when it is added to the dissolving lye.

The amount of formaldehyde used may vary within a range of from 0.05% to 1.0%, based on oven dry recoverable cellulose in viscose (hereinafter abbreviated as CiV). The preferred amount of formaldehyde is 0.5% CiV. While amounts higher than 1.0% CiV may be used, such increased amounts result in no further improvement in the yarn.

The formaldehyde is used in combination with other so-called modifiers in the viscose such as the polyglycols, alkoxylated amines, and their quaternary derivatives. The alkoxylated amines are known in the art as Ethomeens\* and are described in detail in U.S. Patent No. 2,978,292, the disclosure of which is incorporated herein by reference. Their quaternary derivatives are known as

Ethoquads\* and are described in detail in application Serial No. 609,792, filed September 14, 1956, having common ownership herewith. The polyglycol used is preferably either polyethylene glycol or polypropylene glycol, the molecular weight of which may vary depending upon the spinning conditions and the particular amine employed. These modifiers may be present to the extent of 0.3% to 5.0% CiV.

In the preparation of viscose according to this invention, the source of the cellulose may be wood pulp, cotton linters, or a mixture thereof. The cellulose content of the viscose may range from about 5.0%—8.5%. The amount of carbon disulfide used during the xanthation

\*Registered trademarks of Armour and Company.

step may vary from 25-60% CiV, with the preferred amount being 38%-40%. In general, the viscose is aged to approximately the same level of maturity before spinning as that normally used. For example, a 7.3-5.5 (percent cellulose-percent total alkali) viscose may have a Hottenroth maturity index varying at spinning from about 8-20. However, it is preferred to keep the maturity in the 13-14.5 range for best spinnability and properties.

In order to determine proper maturity control, a comparison was made between viscose solutions containing formaldehyde and viscose solutions with no formaldehyde. As is readily apparent from the representative examples set forth in the table below, the addition of formaldehyde to the dissolving lye accelerate the second aging considerably.

TABLE I

|                                      | 0.5% CiV H <sub>2</sub> CO added to the dissolving lye | No H <sub>2</sub> CO added |
|--------------------------------------|--------------------------------------------------------|----------------------------|
| Dissolving end temperature, ° C..... | 16.5                                                   | 16.5                       |
| Second aging, hours.....             | 28                                                     | 43                         |
| Maturity.....                        | 11-13                                                  | 15-17                      |

The effect of formaldehyde on the xanthate ratio as plotted against the maturity index can be seen in the following graph wherein a viscose solution containing 0.5% formaldehyde is compared with a viscose solution containing no formaldehyde.



Viscose prepared in accordance with this invention is extruded into an acid primary bath, from which the filaments thus-produced are withdrawn and highly stretched, preferably in a hot acidic secondary bath. They are then aftertreated in the usual manner. The primary spinbath contains an aqueous solution of from 2%-10% sulfuric acid, 3%-26% sodium sulfate and 1%-9% zinc sulfate. For special purposes, other metal salts may be substituted for the zinc sulfate. Preferably the total salt content should not exceed 15%. In addition, modifiers such as the alkoxyLATED amines may be present in small quantities. Stretching is preferably carried out in a dilute sulfuric acid containing second bath, maintained at a temperature of about 80°-100° C. Small quantities of sodium and zinc sulfates may also be present in this bath. The spinning stretch is preferably adjusted to 1 gram per denier.

The invention will be more clearly understood by reference to the examples and discussions which follow. These examples are given for illustrative purposes only and are not to be construed as limitative. All concentrations used herein unless otherwise designated are calculated as percentages by weight based on the viscose solution or the spinbaths.

## Example I

Alkali cellulose was prepared in the conventional manner from wood pulp and aged to obtain a degree of polymerization that would yield a viscose solution viscosity of 50-60 seconds by the ball fall method. The alkali cellulose was xanthated with carbon disulfide and the xanthate thus obtained was dissolved in a caustic soda solution containing (1) 0.05% CiV formaldehyde added immediately prior to dissolving; (2) 1.5% CiV of an ethoxylated coconut oil amine (available commercially as Ethomeen C-25 from Armour and Company) having the general formula



in which  $n$  is 12 to 14 and  $x+y=$  about 15; and (3) 1.5% CiV polyethylene glycol having a molecular weight of at least 2000. After dissolving, a viscose was obtained having a composition of 7.3% cellulose, 5.5% sodium hydroxide and 2.25% total sulfur. The freshly prepared viscose solution was deaerated, filtered, and ripened to a Hottenroth maturity index of about 13.5.

The viscose solution was extruded into a primary spinbath containing 5.0% H<sub>2</sub>SO<sub>4</sub>, 8.5% Na<sub>2</sub>SO<sub>4</sub>, 5.0% ZnSO<sub>4</sub> plus 1000-2000 parts per million of Ethomeen C-25. The temperature of the spinbath was maintained at 42° C. After a travel of 24 inches through the spinbath, the yarn was withdrawn and passed through a secondary bath containing 3.0% H<sub>2</sub>SO<sub>4</sub>, 1.4% Na<sub>2</sub>SO<sub>4</sub>, and 0.5% ZnSO<sub>4</sub>, maintained at a temperature of 92° C. for an immersion distance of 40 inches. The yarn thus produced was then collected in a rotating pot. A tension of 1600 grams was maintained in the secondary bath to produce a stretch of 140%. The collected yarn was aftertreated in the conventional manner and tested for strength and elongation in both conditioned and wet state. The properties of the yarn are set forth in Table II.

TABLE II

| Yarn produced according to Example I | No. of cakes | Cond. Stgth., g./d. | Cond. Elon., Percent | Wet Stgth., g./100 d. | Wet Elon., Percent | Mod. Cond. | Mod. Wet |
|--------------------------------------|--------------|---------------------|----------------------|-----------------------|--------------------|------------|----------|
| 1698 Denier/1644 Filaments.....      | 9            | 5.51                | 15.6                 | 369                   | 18.1               | 35.3       | 24.0     |

## Example II

Five 7.3/5.5/2.3 (percent cellulose-percent total alkali-percent total sulfur) viscoses were prepared in a manner similar to that described in Example I. One was a control and contained no formaldehyde. The other four contained varying amounts of modifiers. All were aged to a Hottenroth maturity index of 16-20. Samples of each were extruded into spinbaths containing different percentages of H<sub>2</sub>SO<sub>4</sub>. The other additives to the spinbath were held constant at 8.5% Na<sub>2</sub>SO<sub>4</sub> and 5.0% ZnSO<sub>4</sub>. The primary spinbaths were maintained at a temperature of 42° C. with the immersion distance being 28 inches. The secondary baths all contained 2.4% H<sub>2</sub>SO<sub>4</sub>, 1.1% Na<sub>2</sub>SO<sub>4</sub> and 0.5% ZnSO<sub>4</sub>, and were maintained at 92° C. Tension was adjusted to 1100 grams per denier. All yarn samples contained 1100 filaments and averaged approximately 1100 denier.

TABLE III

| Percent<br>$H_2SO_4$<br>added to<br>spinbath | Control, 1.5% <sup>1</sup><br>Ethomeen C-25, 1.5% <sup>1</sup><br>Polyethylene Glycol |                            |      | 0.5% <sup>1</sup> $CH_2O$ , 1.5% <sup>1</sup><br>Ethomeen C-25, 1.5% <sup>1</sup><br>Polyethylene Glycol |                            |      | 0.5% <sup>1</sup> $CH_2O$ , 0.5% <sup>1</sup><br>Ethomeen C-25, 3.0% <sup>1</sup><br>Polyethylene Glycol |                            |      | 0.5% <sup>1</sup> $CH_2O$ , 3.0% <sup>1</sup><br>Polyethylene Glycol |                            |       | 1.0% <sup>1</sup> $CH_2O$ , 1.5% <sup>1</sup><br>Ethomeen C-25, 1.5% <sup>1</sup><br>Polyethylene Glycol |                            |      |
|----------------------------------------------|---------------------------------------------------------------------------------------|----------------------------|------|----------------------------------------------------------------------------------------------------------|----------------------------|------|----------------------------------------------------------------------------------------------------------|----------------------------|------|----------------------------------------------------------------------|----------------------------|-------|----------------------------------------------------------------------------------------------------------|----------------------------|------|
|                                              | Cond.<br>Stgth.,<br>g./d.                                                             | Cond.<br>Elon.,<br>Percent | Mod. | Cond.<br>Stgth.,<br>g./d.                                                                                | Cond.<br>Elon.,<br>Percent | Mod. | Cond.<br>Stgth.,<br>g./d.                                                                                | Cond.<br>Elon.,<br>Percent | Mod. | Cond.<br>Stgth.,<br>g./d.                                            | Cond.<br>Elon.,<br>Percent | Mod.  | Cond.<br>Stgth.,<br>g./d.                                                                                | Cond.<br>Elon.,<br>Percent | Mod. |
| 4.5-----                                     | 4.94                                                                                  | 16.6                       | 29.8 | 4.82                                                                                                     | 15.4                       | 31.3 | 5.02                                                                                                     | 15.4                       | 32.6 | 5.33                                                                 | 17.0                       | 31.3  | 5.47                                                                                                     | 16.2                       | 33.7 |
| 4.75-----                                    | 5.08                                                                                  | 16.5                       | 30.8 | 5.49                                                                                                     | 16.6                       | 33.1 | 5.47                                                                                                     | 15.6                       | 35.1 | 5.28                                                                 | 16.2                       | 32.6  | 5.48                                                                                                     | 16.2                       | 33.8 |
| 5.0-----                                     | 4.92                                                                                  | 15.8                       | 31.2 | 5.57                                                                                                     | 15.4                       | 36.2 | 5.35                                                                                                     | 15.2                       | 35.2 | 5.10                                                                 | 14.9                       | 34.2  | 5.44                                                                                                     | 16.1                       | 33.8 |
| 5.25-----                                    | 4.79                                                                                  | 15.3                       | 31.3 | 5.50                                                                                                     | 15.4                       | 35.7 | 5.32                                                                                                     | 14.5                       | 36.7 | 4.66                                                                 | 12.7                       | 36.7  | 5.26                                                                                                     | 15.1                       | 34.8 |
| 5.5-----                                     | 4.12                                                                                  | 13.4                       | 30.8 | 5.48                                                                                                     | 14.9                       | 36.8 | 4.23                                                                                                     | 11.0                       | 38.5 | -----                                                                | -----                      | ----- | 5.29                                                                                                     | 15.5                       | 34.1 |

<sup>1</sup> All percentages based on cellulose in viscose.

## Example III

Five 7.3/5.5/2.25 (percent cellulose-percent total alkali-percent total sulfur) viscose were prepared using the same procedure as that described in Example I. All were aged to a Hottenroth maturity index of 13-14.5. Viscosity was 50-60° seconds, ball fall method. Different percentages of formaldehyde were used in each sample, the remaining additives being constant at 0.5% CiV polyethylene glycol and 2.0% CiV Ethomeen C-25. Each viscose was extruded into a spinbath containing 5.0%  $H_2SO_4$ , 8.5%  $Na_2SO_4$  and 5.0%  $ZnSO_4$  plus 1000-2000 parts per million Ethomeen C-25. Temperature of the spinbath was maintained at 42° C., with immersion for 24 inches. The secondary bath composition was 3.0%  $H_2SO_4$ , 1.4%  $Na_2SO_4$  and 0.5%  $ZnSO_4$ , with the temperature being 93° C. Immersion distance was 40 inches. Tension and stretch were the same as in Example I. The results were as follows:

TABLE IV

|                                 | Percent CiV Formaldehyde in Viscose |               |               |               |               |       |
|---------------------------------|-------------------------------------|---------------|---------------|---------------|---------------|-------|
|                                 | 0                                   | 0.1           | 0.2           | 0.3           | 0.4           | 0.5   |
| 1700/<br>1444                   | 1697/<br>1444                       | 1701/<br>1444 | 1698/<br>1444 | 1721/<br>1444 | 1699/<br>1444 | ----- |
| Conditioned Strength, g./d.     | 4.81                                | 5.27          | 5.24          | 5.16          | 5.24          | 5.51  |
| Conditioned Elongation, Percent | 14.8                                | 14.9          | 15.2          | 15.6          | 15.6          | 15.5  |
| Modulus (cond.)                 | 32.5                                | 35.4          | 34.5          | 33.1          | 33.6          | 35.5  |
| Wet strength, g./d.             | 3.68                                | 3.72          | 3.68          | 3.40          | 3.68          | 3.69  |
| Wet elongation, Percent         | 17.8                                | 18.1          | 18.4          | 17.7          | 18.1          | ----- |
| Modulus (wet)                   | 20.7                                | 20.6          | 20.0          | 19.2          | 20.4          | ----- |

As the foregoing examples clearly show, a high strength low elongation and high modulus yarn can be prepared in accordance with this invention by incorporating formaldehyde in the viscose. Such procedure eliminates the use of an expensive intermediate bath system. Most important, however, escaping formaldehyde fumes, necessarily present with the intermediate bath system are likewise eliminated.

While preferred embodiments of the invention have been shown, it is to be understood that changes and variations may be made herein without departing from the spirit and scope of the invention as defined by the following claims.

What is claimed is:

1. A process for the production of high strength, low

elongation viscose rayon yarn and like products which comprises extruding a viscose solution containing from 0.05% to 0.5% formaldehyde, based on the cellulose in viscose, prepared by adding the formaldehyde to the dissolving lye for the cellulose xanthate, and from 0.3% to 5.0% of a modifier based on the cellulose in the viscose, said modifier selected from the group consisting of polyglycols, alkoxylated amines, and their quaternized derivatives, into an acid coagulating and regenerating bath, and collecting the yarn.

2. In the viscose process the improvement comprising dissolving the cellulose xanthate crumbs in a caustic soda solution containing from 0.05% to 1.0% formaldehyde based on the cellulose in viscose and from 0.3% to 5.0% of a modifier based on the cellulose in viscose, said modifier selected from the group consisting of polyglycols, alkoxylated amines, and their quaternized derivatives, spinning the viscose into an acid coagulating and regenerating bath and stretching the resultant filaments whereby a high strength, low elongation filamentary product is obtained.

3. In the viscose process the improvement comprising dissolving the cellulose xanthate crumbs in a caustic soda solution containing from 0.05% to 1.0% formaldehyde based on the cellulose in viscose, incorporating from 0.3% to 5.0% of a modifier based on the cellulose in viscose in the resultant viscose solution prior to spinning, and modifier selected from the group consisting of polyglycols, alkoxylated amines, and their quaternized derivatives, spinning the viscose into an acid coagulating and regenerating bath and stretching the resultant filaments whereby a high strength, low elongation filamentary product is obtained.

4. A process for producing high strength, low elongation rayon products comprising dissolving cellulose xanthate crumbs in a caustic soda solution containing from 0.05% to 1% formaldehyde based on the cellulose in viscose and from 0.3% to 5% of a modifier based on the cellulose in viscose, said modifier selected from the group consisting of polyglycols, alkoxylated amines, and their quaternized derivatives, aging the resultant viscose solution, spinning the aged viscose into an acid and coagulating and regenerating bath and thereafter stretching the thus produced product.

## References Cited in the file of this patent

## UNITED STATES PATENTS

65 2,322,981 Ubbelohde \_\_\_\_\_ June 29, 1943  
3,018,158 Mitchell et al. \_\_\_\_\_ Jan. 23, 1962